

Sept. 28, 1926.

1,601,015

J. G. AARTS

## METHOD FOR PRODUCING PIG IRON OR STEEL IN BLAST FURNACES

Filed March 29, 1924 2 Sheets-Sheet 1



Inventor  
J. G. Flatz  
By Marks & Clark  
Prints

Sept. 28, 1926.

1,601,015

J. G. AARTS

# METHOD FOR PRODUCING PIG IRON OR STEEL IN BLAST FURNACES

Filed March 29, 1924

2 Sheets-Sheet 2



## UNITED STATES PATENT OFFICE.

JACOBUS GERARDUS AARTS, OF DONGEN, NETHERLANDS, ASSIGNOR TO AARTS-EISEN  
AKTIENGESELLSCHAFT, OF LUZERN, SWITZERLAND.

## METHOD FOR PRODUCING PIG IRON OR STEEL IN BLAST FURNACES.

Application filed March 29, 1924, Serial No. 702,954, and in Germany May 8, 1923.

My invention relates to an improved method of treating iron ores and ferriferous waste in a blast-furnace in order to produce pig-iron or steel.

5 The blast-furnace process hitherto accomplished is objectionable for several reasons or disadvantages. As coke and iron-ore are supplied to the furnace in successive alternate layers, the two materials cannot mix 10 thoroughly and even in the bottom part of the furnace they mix only very imperfectly.

Further the ore is owing to its pieced or 15 lumpy shape mainly not affected by the carbon monoxide-gas (CO) except externally, that is to say, by contact with its outer faces only, and this is particularly prejudicial in case of hot agglomerated and fritted materials as always present in blast-furnaces even in temperature zones at 1200° to 1300° C.

20 As a result of this incomplete reduction the oxides in the ores, that have not been reduced, go into the slag which is formed in the bottom-zone of the furnace. Ore however, thus slagged or fritted, cannot be read- 25 ily reduced, so that the reduction must be mainly accomplished in the slag. This also refers to objectionable constituents, such as sulphur, arsenic and so on. The iron must be recovered from these compounds which 30 partly are hardly reducible, by the aid of dissolved carbon.

Considering this, the blast-furnace process as hitherto carried out involves, that the main portion of the reducing operation is 35 accomplished in a very restricted space and under unfavourable circumstances, especially in the molten mass where quite a multitude of reactions take place which do not start from metallic iron but from iron oxid and 40 which occur while the reagents are in a liquid state.

Due to the stated unfavourable circumstances the quality of the produced pig-iron is deficient; but a still more objectionable 45 particularity of the old process resides in the excessive consumption of coal or coke, since the principal reaction starts from solid carbon with the intermediate formation of carbon-monoxide and iron-carbide.

50 A further drawback of the old process lies in the fact that all of the reductions

take place in presence of excessive quantities of carbon acting to reduce again directly the formed carbon-dioxid or carbonic acid, the more so as the average temperature in a 55 blast-furnace is above 1000° C., so that carbonic-acid will decompose.

The object of my invention is to remedy all of the hereinbefore mentioned disadvantages of the old art.

I am aware that electrical blast-furnaces have been suggested heretofore, which are provided with a short supplying tube or conduit mounted in the mouth to depend therein so that the fuel may be fed in through said tube, while the ore is supplied separately from the fuel in the annular space surrounding said tube. Obviously as far as the tube or conduit goes, the two materials will descend in the furnace separately for the purpose and with the result of producing in the upper portion of the furnace a coking operation at a low temperature. In contradistinction thereto the essential and novel features of my invention are as follows.

I supply the ore and the fuel, with or without the required additions, to separate spaces in the furnace, said spaces going down as far as the boshes. The gases arising from the boshes act to reduce in a dry 80 way the ores mainly without primary coal being present, whilst the fuel is subjected to fractional distillation and coked. The ores and the fuel having thus undergone an introductory or partial reduction each of its 85 own, thereafter meet on the hearth where the final or complete reduction of the ore, including manganese, silicon and so on, takes place, the metallic iron and the slag are melted and at the same time the iron is car- 90 buretted.

It will be seen that in my improved method the reduction of the ore and the coking of the fuel to a large extent or mainly are brought about in an operation separate from 95 the melting operation, so that the process is carried out under circumstances which are especially advantageous for obtaining a pure product of better quality. The amount of fuel supplied at the top of the furnace may 100 be a multiple less, with relation to each ton, than the weight of the ore whereby a con-

siderable saving in fuel is realized. If desired or required the impurities, such as sulphur and arsenic, present in the charge may be hydrogenized and volatilized, with the aid of the hydrogen produced in the process, in the middle and lower part of the ore column and in absence of any coal, so that such impurities are prevented from going into the iron.

10 In the accompanying drawing wherein an approved embodiment of the invention is illustrated:

Fig. 1 shows a vertical section through the complete furnace,

15 Fig. 2 is a vertical section through the furnace with means for feeding the fuel and the ore and conveying means for causing the ore to travel through the furnace.

20 Fig. 3 shows several cross-sections through the furnace namely along lines A—A, B—B, C—C, D—D of Fig. 2.

25 Fig. 4 is a diagrammatic longitudinal section through the furnace showing the temperatures for the zones at the various heights of the furnace.

Coaxially to the vertical axis of the furnace is an inner shaft or chamber *b* within a larger shaft or chamber *a* of annular shape, the former receiving the fuel and the latter being supplied with the ore, both with the required additions. The interior of the furnace thus comprises four zones I, II, III and IV, I being the melting zone, II being the coke generator, III being the ore shaft and IV being the fuel shaft. The raw fuel, with additions if required, is fed at the top of the vessel *c*, Figure 2, and the ore with additions, if required, is fed into the surrounding funnel *d*, and the supplied fuel and ore are conveyed from the funnel *c* and the funnel *d* to the fuel shaft and the ore shaft respectively through descending tubes *f* and *g* provided with suitable closures.

40 Obviously the blast-furnace may, if desired, comprise a plurality of such reducing and coking chambers independently of each other. The ore chamber III may be equipped, wholly or partially, with mechanically working conveying devices, such as rotary scoops or shovels for continuously transporting the ore from one story to the next lower story in counter-current to the gases rising in wavy lines.

45 In the chamber IV the fuel gradually descends and in doing so it is subjected to fractional distillation and coked by the heat of the rising gases, as will be described hereinafter more in detail. The ore and its additions, if any required, are supplied at the top of the reducing chamber III and gradually moved downwards in said chamber. During this gradual downward movement the ore is wholly or mainly reduced just in accordance with its particular nature.

In order to retain the descending ores within the reduction zone as long as possible and to bring them in constant and most intimate contact with the ascending gases, the reduction room is equipped with stories of staggered or overlapping relationship, so that the gases are compelled to move in permanent counter-current with respect to the descending ores, the arrangement being such that the so-called dry reduction of the ores and the expulsion of certain objectionable impurities will be ensured thereby.

The reduced and purified ores travel from the lower end of the ore shaft having a bottom *k* for supporting the weight of the ore through the openings *l* of said bottom into the chamber II in order to meet and be mixed with the coked fuel descending from the fuel shaft IV. In said chamber II the reduction of the ores is completed, the iron and slag melted and the iron carburetted, as far as such is required. The hearth is provided, as usually, with a slag, hole *m*, a tapping hole *n* and air-blast nozzles *o*.

50 The ore on having been wholly or mainly reduced in the dry reduction chamber III at a temperature below 1000° C., mixes, still finely comminuted, with the coke in the shaft or chamber II and is completely reduced to ferrite, carburetted and melted down in the latter. The reduction of the metallic oxides on the one side and the reduction of the impurities, on the other hand, therefore, occur separately and under different physical conditions, that is to say, the former in a dry way and the latter in a melted state, it being noticeable that the principal impurities such as sulphur and arsenic, have been previously removed from the ore in a dry way in the chamber or shaft III as will be hereinafter described more in detail.

55 It is advisable to inject steam through the radially arranged or distributed pipes *p* into the lower part of the fuel shaft or chamber IV, which part is heated above 1100° C. The steam rises within the chamber IV together with the carbon-monoxid gases ascending from the hearth II and produces on meeting the incandescent fuel water-gas. Instead of steam or together therewith, if required or advisable in the particular conditions of the case, waste-gases containing carbonic acid and discharged from the ore shaft or chamber III through the openings *q* may be introduced into the fuel shaft IV at the bottom thereof for the purpose of reducing the carbonic acid contained therein and to regenerate the said waste-gas.

60 Further it will be advisable to introduce the gas discharged from the shaft IV through the openings *r* after separation from its valuable constituents, into the shaft III.

after cooling, by means of the conduits *t*. The gases coming from the hearth must partly be employed for the reduction of the ore, but they have a temperature of between 1400 and 1500° C., which is too high for the ores, since the latter would be fritted and the slag melted thereby. It, therefore, is necessary to reduce the temperature of the gases and for this purpose I utilize in my improved method mixed gas issued from the coking chamber and purified, which does not contain any by-products.

In this manner I also realize the important advantage of having a gas rich in hydrogen and oversaturated with carbon in the reduction chamber. Hydrogen combines with sulphur, arsenic and the like and the gaseous compounds thus formed are carried away with the gas current. Moreover the hydrogen greatly assists in the reducing process and just in this point my improved method is essentially distinguished from the customary blast-furnace method, for hydrogen is the most efficient reducing agent known in the art.

As the reduction of the ores is of great importance and a characteristic feature of my new method, I deem it necessary to explain in detail the single operations thereof.

The hot carbon-monoxid gases rising from the lower part of the furnace are mixed with the cool gases derived from the by-product, recovery for the reasons hereinbefore mentioned, whereby, as above explained, a practically carbonic acid-free gas rich in hydrogen and oversaturated with carbon will be obtained, which comes in contact with the already reduced ores at a temperature of 950° C. The hydrogen which, as is known, acts as a reducing agent even at low temperatures, did already create metallic iron in the upper zones of the reduction shaft. Upon meeting a gas rich in carbon-monoxid and containing hydrocarbon this gas will act as a catalyst and the catalyzing action will be very efficient owing to the enormous constantly increasing and varying surface of the gas. Amorphous carbon precipitates upon the metallic iron, and, as such carbon forms at a low temperature, it is evidently  $\alpha$ -carbon of highest activity and of carbureting property. The thus formed iron-carbid- $\text{Fe}_3\text{C}$  is a still more active or efficient reducing agent and adapted to reduce, together with the said  $\alpha$ -carbon present, the iron and oxygen compounds still existing below the metallic surface of the ore. In this way carbonic acid respectively carbon-monoxid forms, while the iron carbid is reduced to metallic iron, which in turn acts as a catalyst and again receives active carbon. This circuit action continues until the ore particles are completely reduced. As the ore advances to the higher temperature-zones, the less active  $\beta$ -carbon forms at temperatures above

600° C. acting to carburet the iron preliminarily and to protect the same from subsequent melting with the slag.

My improved blast-furnace method may be divided into four separate elements according to the four zones I to IV of the furnace (see Figure 4):

(1) *The lower hearth.*—In the lower-hearth the molten mass or bath consisting of iron and slag is intended to be brought to a temperature of about 1500° C. and maintained at such temperature, until the mass is discharged by tapping. Over and above the bath the oxidizing zone of the hot vent prevails which, however, cannot exert an oxidizing action to any noticeable degree on account of the great speed of the dropping metal.

(2) *The upper-hearth.*—In this part of the furnace the following operations shall take place, viz.

(a) The final reduction, if any required, of the ore with the aid of solid carbon at temperatures above 1000° C.

(b) The melting of the metal and of the slag.

(c) The carburetting of the liquid iron at temperatures of between 1200° to 1500° C.

(d) The formation of the carbon-monoxid gas.

(3) *The reduction chamber.*—In this part of the furnace the following operations are to occur, viz.:

(a) The dry reduction of the ore with the aid of the described gas mixture at a temperature not above 950° C.

(b) The hydrogenization of the impurities of the ore, in particular of sulphur and arsenic, as above described.

The reduction chamber, if constructed to be of annular shape, is further designed with a view to avoid any losses of heat from the coking chamber through radiation;

(4) *The coking chamber.*—In this part of the furnace the following operations take place, viz.:

(a) The fractional distillation of the fuel at a temperature gradually rising from the temperature of the atmosphere up to 1300° C.

(b) In the lower part of the shaft, where the temperature is between 1100° and 1300° C., the production of water-gas and the reduction of the temperature to the limit suitable for a satisfactory coking process.

(c) In case that conditions allow, the regeneration of a part of the gas discharged from the shaft and introduced at the bottom of the coal shaft, or of foreign gases of the kind, either alone or together with the production of water-gas at temperatures of 1100° to 1300° C.

In this regard it is to be noted that the distillation of the coal takes place endothermically i. e. in a heat consuming manner,

until the temperature in the lower zone of the coal reaches 600° C. Thence the distillation is exothermic i. e. heat producing.

The advantages of my improved methods 5 are as follows:

(1) A separate coking plant may be dispensed with so that the considerable costs of the erection thereof, repairs and management are saved;

10 (2) Saving of losses of heat arising from reheating and drying the coke in the blast-furnace;

(3) Saving of losses arising from cooling, loading, piling, transporting and charging the coke;

(4) Saving of cost for transporting or conveying materials from the coke oven to the furnace;

20 (5) Avoiding deterioration of quality of the coke at the pressing, loading, transporting and charging operations;

(6) The coal to be coked is heated, without any expense and without combustion of gas by the large amount of the available hot 25 gases, so that the gases otherwise required for heating the coke oven are available for other purposes; moreover they bring about an absolutely ideal distillation by preserving all of the distillates, no matter whether obtained at high or at low temperatures, and preventing their premature liquefaction or decomposition; in this way the output is greatly increased, as regards both quantity and value thereof, a fact which 30 further assists in lowering the price of the coke going into the furnace and of the iron produced.

(7) The method is restricted to the recovery from the waste-gases of the coking 40 chamber of ammonia and of those hydrocarbons, which when cooled are liquid and to the desulphurization of said hydrocarbons, if required. In this way a gas is obtained which is practically free from carbonic acid, 45 poorer than normally in nitrogen, rich in hydrogen and over-saturated with carbon. A gas of this sort is a most efficient reducing agent for iron ores and a most efficient carburetting means for metallic iron, but 50 it has never been used or available in the art as hitherto practiced.

For hydrogen is a reducing agent which 55 is not only by far more efficient than carbon-monoxid, but also active at lower temperatures as compared with the latter, and further hydrogen acts to combine with very objectionable impurities, such as sulphur and arsenic, forming gaseous compounds therewith, which are easily removed, so that 60 iron of greater purity and higher value will be obtained.

Moreover owing to the enrichment with carbon monoxid and hydrocarbon an over-saturation with carbon is obtained so that

active, amorphous carbon may be formed 65 in abundance which will act to greatly promote the reduction of the iron-oxygen-compounds even at low temperature;

(8) The coke need not be of a certain high quality, since it has not to support the 70 heavy weight of the ore and additions. Consequently the coke is not subject to crushing and rubbing, so that also coal of less value may be employed in the furnace;

(9) In order to ensure a ready, quick and 75 thorough reduction of the ores at low temperature, the ores must be finely comminuted. Considering this, there now is a possibility of utilizing ores on stock, which at the present state of the art, cannot be used for the purpose on account of their pulverulent state, or which otherwise must be previously briqueted in order to be in a treatable state, which, however, involves considerable extra costs;

85 (10) By causing the just mentioned rich and cold waste or by-product gases to mix with that portion of the carbon-monoxid containing gases coming from the upper hearth, which is intended to flow through the reduction chamber and which is of a detrimentally high temperature involving the danger of the ore particles getting coated with a layer of fritted or molten slag impermeable to the gas, a considerable reduction 90 of the temperature is ensured, which will remove such danger. Apart from that the reduction of the ore particles commences, owing to the presence of reducing agents, which are even active at low temperature, in the upper stories of the reduction chamber and immediately thereafter the carburation of the produced metallic iron begins.

100 (11) Not only the costs of the unnecessary coking plant are fully saved but also the costs to be invested in erecting the blast-furnace are considerably reduced. In furnaces of the kind hitherto constructed 105 enormous quantities of the very voluminous coke must slowly move down from the top to the bottom of the furnace, before the coke is in the required state of combustion, for the reason that the coke is charged together 110 with the ore in alternate layers and cannot advance except in dependence upon the speed of the movement of the ore.

115 In my improved method, however, the descending movements of the two materials are independent of each other and the fuel is free to move down at a greater speed. Consequently the portion of the furnace required for the reception of the fuel is comparatively small, which involves a considerable reduction of the costs to be invested 120 in the construction of the furnace.

125 (12) All of the aforementioned savings in fuel involve further reduction of the

room required for the fuel, and particularly an enormous reduction of the cost of production of the iron.

From the foregoing, it is believed, that 5 the advantages and novel features of my invention will be readily understood and, therefore, further detail description is deemed unnecessary.

It will be evident, however, that my invention may be varied and adapted in many 10 ways, according to the several requirements desired, or most suitable under the different circumstances.

What I claim is:

15 1. A method of producing iron in a blast furnace, consisting in feeding the ore in some cases with additions downwardly through the blast furnace in an ore shaft and out of contact with solid fuel, feeding the 20 fuel downwardly through the furnace in a fuel chamber, subjecting the fuel to fractional distillation and coking in said chamber, passing steam into the lower portion

of the fuel chamber, supplying gas from the upper part of the fuel chamber to the 25 lower portion of the ore shaft for reducing the grains of ore to iron sponge, and bringing the reduced ore into contact with the coke produced in the fuel chamber in the bosh of the furnace so as to melt down the 30 iron and simultaneously carburize it.

2. A method of producing iron as claimed in claim 1, characterized by the feature that the temperature of the gases serving for carrying out the reduction process is fixed 35 by mixing the cooled gas derived from the fuel shaft with the hot gases which rise from the melting zone of the furnace.

3. A method of producing iron as claimed in claim 1, characterized by the feature that 40 simultaneously with the steam, a portion of the gases which pass out of the reduction shaft is introduced into the fuel shaft.

In testimony whereof I affix my signature.

JACOBUS GERARDUS AARTS.